

Aug. 23, 1949.

W. S. RICE

2,480,048

CASTING PROCESS

Filed July 10, 1944



INVENTOR.

William S. Rice.

BY

Crown, Jackson, Bottcher & Diers  
Atty's.

## UNITED STATES PATENT OFFICE

2,480,048

## CASTING PROCESS

William S. Rice, Chicago, Ill.

Application July 10, 1944, Serial No. 544,265

4 Claims. (Cl. 18—55)

1

This invention relates to casting, and has to do with a casting process employing a low fusing mold which may readily be removed from the article cast therein so as to avoid injury to the cast article, such as might occur if the mold were removed from the article by chopping or breaking the mold as is done in casting articles in refractory molds.

My invention is directed to a casting process in which I provide a low fusing mold, this mold having therein a casting cavity conforming to the desired article to be cast, the mold, after casting of the article therein, being removed, conveniently by melting, so as to separate the material of the mold from the cast article without injury to the latter. In the more specific and preferred form of my process, disclosed herein by way of example, I provide a mold formed of a metal fusible at a temperature which will not cause injury to or impairment of the article cast therein, and fill the cavity of the mold with a suitable material, conveniently a material of a character to be heat cured and to set at a temperature lower than the fusing temperature of the metal of the mold, the mold with the material therein being then heated to a proper temperature to cause curing and setting of the material, after which the mold is heated to a higher temperature effective to cause fusing thereof without injury to the cast article, thereby melting the mold away from the article cast therein. Further objects and advantages of my invention will appear from the detail description.

In the drawings:

Figure 1 is a side view of a human ear illustrating the first step of the process of my invention, which consists in taking an impression of the ear cavity;

Figure 2 is a sectional view through a retaining ring disposed about the impression produced by the step of Figure 1, this impression serving as a pattern about which the low fusing material which constitutes the mold is poured;

Figure 3 is a sectional view through the mold produced by the operation of Figure 2, with the mold cavity filled with a casting material of a character to be heat cured and to set when cured, the mold with the cavity thereof filled with the casting material being subjected to heat treatment at a temperature below the fusing or dissolving temperature of the mold, there being a cover on the mold to protect the casting material from the heating medium;

Figure 4 is a view similar to Figure 3 but illus-

2

trating the step of removing the mold by fusing thereof away from the cast article;

Figure 5 is a side view of the cast article remaining after fusing of the mold;

Figure 6 is a sectional view, with the article to be reproduced shown in elevation, illustrating the first step of the process of my invention as applied to producing a cast of a tooth, this first step consisting in making an impression of the tooth;

Figure 7 is a sectional view, partly in elevation, illustrating the second step consisting in making a casting from the mold produced by the operation of Figure 6;

Figure 8 is a sectional view, partly in elevation, of a ring disposed about the casting produced by the operation of Figure 7, illustrating the step of pouring the low fusing material from which the mold is to be formed about the casting as a pattern;

Figure 9 is a sectional view of the mold produced by the operation of Figure 8, with the mold cavity filled with a casting material of a character to be cured and to set when subjected to heat treatment at a temperature lower than the melting temperature of the mold, illustrating the step of heat treating the material in the mold cavity;

Figure 10 is a view similar to Figure 9 but illustrating the step of melting the mold from about the article cast therein; and

Figure 11 is a side view of the article cast in the mold after the mold has been melted from the cast article.

In applying devices to aid deaf people in hearing, commonly termed hearing aids, it is important that the instrument which goes into the ear fit the ear cavity accurately and comfortably so as to be retained in proper position therein and not cause undue discomfort to the user. Under present practice considerable delay in fitting such devices is incurred due to the necessity of having the patient present for the fitting, which also frequently causes considerable loss of time by the patient. By making an accurate reproduction of the patient's ear cavity and shaping the instrument which goes into the ear accurately in accordance with this reproduction, an accurate and comfortable fit of the instrument can be assured and the delay incident to waiting until the patient is available for fitting the instrument to his ear, as well as the loss of the patient's time, can be avoided. In Figures 1 to 5, inclusive, I have illustrated the process of my invention as applied to casting an article, in the nature of a plug, corresponding accurately to the cavity of a person's

ear, this article serving as a guide in constructing an instrument to be fitted into the ear, by means of which the instrument can be so formed as to provide for an accurate and comfortable fit.

In Figure 1 an impression of the cavity of a person's ear  $e$  is taken by inserting into the ear a suitable known impression material  $12$ , this operation being performed in a known manner, and any suitable impression material which when set will retain the shape into which it has been formed may be used. For example, an impression plaster composition may be used, though I preferably use the impression material known commercially as "Coeloid" made by Coe Laboratories, Inc., of Chicago, Illinois. The latter impression material—"Coeloid"—after it has set sufficiently to retain the shape to which it has been formed possesses appreciable elasticity, which is desirable in certain cases as will be explained later.

The impression taken as in Figure 1 produces a plug shaped article  $13$ , shown in Figure 2, conforming to the ear cavity from which the impression is taken. After this article  $13$  has taken its complete set it is placed flatwise upon a flat supporting surface, as in Figure 2, and a retaining ring  $14$ , formed of a metal or alloy having a high fusing temperature, is placed upon the supporting surface about the article  $13$ , which serves as a pattern. The ring  $14$  is then filled to a suitable depth with a material  $15$  which may readily be removed, conveniently by application of heat at a suitable temperature to cause melting or fusing of the material  $15$ , this material serving as an investment for the article or pattern  $13$  and being of a character to set about the same and within the ring  $14$ . Conveniently the material  $15$  is an alloy consisting of 41.67% tin, 16.67% lead and 41.66% bismuth, having a fusion point of 212° F. Alternatively, an alloy consisting of 50% lead, 30% tin and 20% bismuth, having a fusion point of 202° F. may be used. The molten alloy is poured from a suitable crucible or ladle  $16$  into the ring  $14$ , as illustrated, it being understood that the material of which the plug or pattern  $13$  is formed is of such character as not to be impaired or in any way injuriously affected by the molten alloy with which it is invested. After the investment material or alloy  $15$  has set, the pattern  $13$  is removed therefrom, by breaking the pattern and removing the parts thereof where necessary, if this pattern be formed of plaster or other non-elastic material, or if the pattern be formed of a material which when finally set possesses appreciable elasticity, of which there are known materials including "Coeloid" above referred to, the pattern may be removed as a unit. That provides a mold comprising a heat destructible body formed of the material or alloy  $15$ , within the ring  $14$ , having therein a casting cavity conforming accurately to the pattern  $13$ . The alloy used should be such as not to have objectionable dimensional change in cooling from its melting point to room temperature, as will be understood by those familiar with the casting art, and the retaining ring  $14$  preferably should be of a metal or alloy having a fusion point or temperature considerably above that of the investment alloy.

After the mold has been produced in the above manner, the cavity thereof is filled with a suitable material for producing the desired cast article. This casting material should be a settable material of such character as to fill completely and accurately all portions of the casting cavity in the mold and not to be impaired or injured

at temperatures required to destroy or dissolve the mold away from the cast article. Preferably, I employ a casting material which may be cured and will set at a temperature appreciably lower than the fusing temperature of the mold and which, when cured and set, has a fusing temperature sufficiently higher than that of the mold so that it will not be softened to an objectionable extent or otherwise impaired or injured in the melting of the mold. I have found that an acrylic resin is well suited for the casting material. The resin which I preferably use is methyl methacrylate, which I mix in powder form with a suitable liquid, such as acrylic acid in its monomer form, to provide a plastic mix of suitable consistency for packing into the mold cavity so as to enter into and completely fill all of the portions thereof. In Figure 3 the mold is shown with the cavity thereof filled with casting material  $18$ , such as that above referred to, or any other suitable material, after which the top of the mold is covered so as to be effectively closed by a slab or plate  $19$  of considerable thickness seating upon the upper end of the mold so as to close the latter, particularly the upper end of the mold cavity, and retain the casting material  $18$  therein. The mold, with the contained casting material and closed by the slab  $19$ , is then immersed in a body of a suitable liquid  $20$ , conveniently water, within a container  $21$ , the mold seating at its lower end upon a grate  $22$  of suitable height resting upon the bottom wall of the container. The liquid  $20$  within the container  $21$  is then heated in any suitable manner, as by means of a burner  $23$ , to a temperature below the fusing temperature of the mold but sufficiently high to heat the mold and the casting material therein to the curing temperature of the latter, which is from 160° F. to 180° F., when using the methyl methacrylate composition above mentioned. During this curing operation, the cover  $19$  seals the upper end of the mold against access of water to the casting material and also prevents escape of the latter from the mold cavity. The material  $18$  tends to expand somewhat during the curing operation and, since it is restrained against escape from the mold cavity by the cover  $19$ , it is cast under pressure which is desirable as assuring accurate reproduction of the fine details of the mold cavity.

After the material  $18$  has been cured and has set, it will not be injuriously affected by the liquid or water  $20$ , it being understood that the liquid used as a heating medium is of a character not to injure the material  $18$  after curing and setting thereof. The cover  $19$  may then be removed or not, as desired, and the temperature of the water  $20$  is then increased sufficiently to cause melting of the mold so as to free the cast article  $24$ , as shown in Figure 4 in which the major portion of the mold has been melted. The material of the mold, as it is melted, passes downwardly through the grate  $22$  into the lower portion of the container  $21$ , and when the mold has been completely melted the article  $24$  rests upon the grate and is completely freed of the material of the mold. It will be seen that the curing operation and the operation of melting the mold may be performed as, in effect, a continuous operation, which is conducive to expedition and facility in casting the article and freeing it from the mold. By melting the mold from about the cast article, risk of injury to the latter is avoided and the article as cast conforms accurately to the pattern about which the mold was

formed. The cast article may then be treated with acid solution, or in any other suitable manner, for removing any dross that may remain thereon, the finished article 24 then appearing as in Figure 5. This article is an accurate reproduction of the original impression or plug and may safely be relied upon in making an instrument to fit into the ear from which the original impression was taken, with assurance that an instrument conforming to the cast article 24 will fit accurately and comfortably into the ear from which the impression was taken and will be properly retained therein.

Since the impression taken in Figure 1 is a positive impression, that is an impression of the inside of the ear, that impression may be used directly as the pattern for forming the corresponding cavity in the mold. Where a negative impression is originally taken, for example the impression of a tooth, it is necessary to make a positive of the impression, which positive is then used as a pattern for forming the cavity in the mold. The process in the latter case is essentially the same as that above described, with the exception of the preliminary steps for obtaining the pattern for use in producing the mold.

Referring to Figures 6 to 11, inclusive, in Figure 6 I have illustrated the steps of taking an impression of a tooth, such as a molar 25 in a mold 26, preferably formed of "Coeloid," though this mold may be formed of any other suitable known impression material which when set possesses sufficient elasticity to permit of removal of the tooth 25 from the mold without adversely affecting the accuracy of the impression therein. The mold 26 is of cylindrical form and, after this mold has set, it is placed within a suitable retaining ring 27 fitting closely about the mold and extending a suitable distance there above, the underface of the mold and the lower end of the ring resting upon a suitable flat supporting surface. The cavity of the mold 26, and the ring 27 to a suitable height above the mold, are then filled with a suitable impression material in liquid form, which when set is elastic but sufficiently rigid to retain its form into which it is shaped by the mold cavity, this material being poured into the mold cavity and the ring from a suitable container 28, as shown in Figure 7. In that connection, no difficulty arises from using the same material for the mold 26 and for producing therefrom the desired pattern, since this impression material—"Coeloid"—when set, will not adhere to the same material poured in contact therewith. Any other suitable impression material may be used, if desired, for forming the desired pattern or model from the mold 26. After the impression material which has been poured into the cavity of the mold 26 and into the ring 27 has set, the resultant model, comprising a disc-shaped plate 30 and a pattern 31 integral with and projecting from the plate 30, conforming to the cavity in mold 26, is removed from this mold, that being permitted by the elasticity of mold 26 and, preferably, of the mold material of which the pattern is formed.

After the pattern has been produced in the manner above explained, it is placed upon a suitable flat supporting surface with the pattern 31 disposed upward, and a retaining ring is then placed about the base plate 30, fitting snugly thereabout with its lower end in contact with the supporting surface, the pattern 31 being disposed centrally within the ring as shown in Figure 8. The pattern is then invested with a low

fusing material, such as the alloy above referred to, poured into the ring from the ladle or crucible 16, as before. After the investment material 15 has set, the pattern 31 is removed therefrom providing a low fusing mold having therein a casting cavity conforming accurately to the pattern 31. This cavity is then filled with a casting material, such as the methyl methacrylate composition above described. The top of the mold is then closed by a cover 19 of considerable weight, as and for the reasons above set forth. The mold, with the contained casting material, is then heated to proper temperature for effecting curing and setting of the casting material, and the mold is then melted away from the cast article. In Figure 9 the casting material is indicated by the reference number 18<sup>a</sup>, since the shape of the mold cavity is different than in Figure 3, though it will be understood that the casting material is the same, or may be the same, in both cases.

Instead of heating the mold and the contained casting material in liquid, the mold may be passed upon a traveling grate 33 moving at appropriate speed through a furnace 34 of any suitable known construction. This furnace 34 has graduated heating zones, as is known, such that during the first portion of the travel of the mold through the furnace the mold is heated to a proper temperature for effecting curing and setting of the casting material 18<sup>a</sup>, while avoiding heating of the mold to a sufficiently high temperature to cause objectionable softening or fusing thereof. After completion of the curing and setting of the material 18<sup>a</sup>, the mold passes into the higher temperature zone of the furnace, where it is heated to a sufficiently high temperature to cause melting of the mold, thereby melting it away from the cast article, the melted material of the mold passing downward through the grate 33 into a suitable trough or tray 35 so disposed that the mold passes thereabove during the operation of melting the material of the mold. The cast article thus freed from the material of the mold rests upon the grate 33 from which it may be removed, the melting operation for removing the body of the mold being shown in Figure 10, in which the major portion of the mold has been melted away. The cast article from which the mold has been removed may then be treated with acid, or in any other suitable manner, to remove therefrom any remaining dross, and then appears as in Figure 11, the article 36 accurately reproducing the pattern 31 and, therefore, accurately reproducing the original tooth 25.

Heating of the mold in water, particularly for melting the mold, is advantageous as preventing objectionable oxidation of the alloy which may be recovered and reused for succeeding molds. It will be understood, however, that the mold may be heated in any suitable manner and, where desired or necessary, such heating may be effected within a suitable atmosphere to prevent oxidation or other action on the mold material such as would interfere with its being reused.

In the production of impressions or plugs, as above described, these articles are unique or individual to the persons from which the impression has been taken and, since ordinarily but one cast article is required, there is no particular reason for retaining the mold which may be destroyed for the purpose of removing the cast article therefrom, as above explained. Likewise, 75 in the casting of teeth and other articles which

are to be retained as reference samples, there is no particular reason for retaining the mold. It will be understood, however, that the casting process of my invention may be used to advantage in cases where it is desired to reproduce 5 an article in considerable numbers, and provides an inexpensive and high speed casting method for that purpose.

In general, the method of my invention comprises forming a mold of a low fusing material, such as an alloy or other material which may be destroyed by the application of heat or in any other suitable manner, and casting in this mold, from a suitable material, the desired article, the mold being then melted so as to free the 10 cast article without risk of injury thereto, such as might occur if the mold were removed from the cast article by breaking up or cutting away the material of the mold.

I claim:

1. The steps in the method of making an article of the class described, which comprise forming a mold body of relatively low fusing metal about a pattern and subsequently removing said pattern to leave a mold cavity, filling said cavity with a material curable at a temperature below the relatively low fusing temperature of the mold body, heating the mold body and the material in said cavity to a temperature sufficiently high to cure said material and to form a cured article but below the fusing temperature of the mold body, and thereafter as a continuous process with said curing operation increasing the heat to heat the mold body to its fusing temperature to melt the same but below the temperature which will deleteriously affect the cured article.

2. The steps in the method of making an article of the class described, which comprise forming a mold body of relatively low fusing metal about a pattern and subsequently removing said pattern to leave a mold cavity, filling said cavity with a material curable at a temperature below the relatively low fusing temperature of the mold body, heating the mold body and the material in said cavity to a temperature sufficiently high to cure said material and to form a cured article but below the fusing temperature of the mold body, thereafter as a continuous process with said curing operation increasing the heat to heat the mold body to its fusing temperature to melt the same but below the temperature which will deleteriously affect the cured article, and permitting the molten mold material to flow away from the cured article during the application of the heat for melting the mold body.

3. The steps in the method of making an article of the class described, which comprise forming a mold body of relatively low fusing metal about a pattern and subsequently removing said pattern to leave a mold cavity opening from one side of the mold body, filling said cavity with a resinous material curable at a temperature below the relatively low fusing temperature of the mold body and which tends to expand when heated to cure the same, applying closure means

over the open side of said cavity, heating the mold body and the material in said cavity to a temperature sufficiently high to cure said material to form a cured article and to cause said resinous material to tend to expand but below the fusing temperature of the mold body, utilizing said closure means to restrain said resinous material against escape from the mold cavity during the curing operation whereby to mold said resinous material under pressure, thereafter as a continuous process with said curing operation increasing the heat to heat the mold body to its fusing temperature to melt the same but below the temperature which will deleteriously affect the cured article, and permitting the molten mold material to flow away from the cured article during the application of the heat for melting the mold body.

4. The method of making an article of the class described, which comprises forming a pattern of the article, placing the pattern on a supporting surface, placing a retaining ring upon the supporting surface about said pattern, introducing to suitable depth in said ring and about said pattern a molten metal fusible at a relatively low temperature to form a mold body and allowing same to set, removing the pattern from said mold body to form a mold cavity therein, filling said cavity with a material curable at a temperature below the relatively low fusing temperature of the mold body and adapted to constitute the body of the finished article, placing the ring having therein the mold body with said last mentioned material in the mold cavity thereof in inverted position upon a grate, heating the material in said cavity to a temperature sufficiently high to cure said material to form a cured article but below the fusing temperature of the mold body, thereafter as a continuous process with said curing operation increasing the heat to heat the mold body to its fusing temperature to melt the same but below the temperature which will deleteriously affect the cured article, and permitting the molten mold material to flow away from the cured article during the application of the heat for melting the mold body.

WILLIAM S. RICE.

#### REFERENCES CITED

50 The following references are of record in the file of this patent:

#### UNITED STATES PATENTS

| Number       | Name             | Date           |
|--------------|------------------|----------------|
| 55 720,482   | Richards         | Feb. 10, 1903  |
| 935,254      | Gleason          | Sept. 28, 1909 |
| 1,087,974    | Owen             | Feb. 24, 1914  |
| 1,135,962    | Aylsworth        | Apr. 13, 1915  |
| 1,343,191    | Allcutt          | June 15, 1920  |
| 60 1,523,519 | Gibbons          | Jan. 20, 1925  |
| 1,796,470    | Meyer            | Mar. 17, 1931  |
| 1,822,285    | Hagman           | Sept. 8, 1931  |
| 2,017,216    | Marcus           | Oct. 15, 1935  |
| 2,203,421    | Stevenson et al. | June 4, 1940   |
| 65 2,249,890 | Droge            | July 22, 1941  |